

## UNITED STATES PATENT OFFICE.

RICHARD G. WOODBRIDGE, OF WILMINGTON, DELAWARE, ASSIGNOR TO E. I. DU PONT DE NEMOURS & COMPANY, OF WILMINGTON, DELAWARE, A CORPORATION OF DELAWARE.

## PROCESS OF TREATING PYRO SMOKELESS POWDER.

No Drawing.

Application filed March 13, 1922. Serial No. 543,475.

*To all whom it may concern:*

Be it known that I, RICHARD G. WOODBRIDGE, a citizen of the United States, and a resident of Wilmington, in the county of 5 New Castle and State of Delaware, have invented a certain new and useful Process of Treating Pyro Smokeless Powder, of which the following is a specification.

This invention relates to the treatment of 10 "pyro" smokeless powder for the purpose of reducing the viscosity-characteristic thereof, thereby making practicable the use of the powder as an ingredient of coating compositions.

15 By pyro smokeless powder, or pyro powder, is meant that grade of smokeless powder made from nitrocellulose almost completely soluble in a mixture of two parts by volume of ether to one part of ethyl alcohol and having a nitrogen content of about 12.60%. When the World War terminated in the year 1918, there existed large surplus stocks of this "pyro" powder originally containing about 0.5% of diphenylamine.

20 Some of this powder is not suitable for use in arts other than the explosive art because the powder grains are difficultly soluble in the usual pyroxylin solvents on account of their relatively large size, but more especially on account of the powder grains giving very viscous solutions. For some uses, the presence of the diphenylamine is objectionable because the diphenylamine reacts with the decomposition products of the 25 powder forming colored nitroso and nitro derivatives and mixed nitroso-nitro derivatives, besides other colored derivatives, the identity of which has not been fully established. Thus, pyroxylin solutions containing

30 diphenylamine are unsuitable except for use in very dark colored products, although diphenylamine itself is an excellent stabilizer and, were it not for its highly colored derivatives, might be a very desirable ingredient of pyroxylin solutions. Another 35 objection is that the presence of diphenylamine in pyroxylin solutions causes a reduction in their viscosities to take place at a faster rate than that when diphenylamine is absent. For many purposes this is not objectionable, but it may be very objectionable when considerable time elapses between the preparation and the use of the pyroxylin 40 solution.

I have discovered that by a prolonged 55 heating of pyro powder while immersed in an organic liquid which is substantially a non-solvent for the powder, such as ethyl alcohol, toluene, etc., the powder may be so changed as to impart to its solutions a 60 much lower viscosity than that of corresponding solutions made from untreated powder. My new process comprises immersing the powder grains in a liquid of the kind 65 above-described and heating the mass, preferably at, or near, the boiling point of said liquid.

In place of the above mentioned non-solvents for pyro powder, I may use another alcohol such as propyl alcohol, or butyl 70 alcohol, or another benzenoid hydrocarbon such as benzene or xylene, or a large number of other liquids, but I prefer to use those liquids, such as ethyl alcohol, which are not only non-solvents for pyro powder, but 75 which when heated are excellent solvents for diphenylamine, and have also considerable, if not excellent, solvent action for the nitroso and nitro derivatives of diphenylamine.

I do not confine myself to the use of a 80 single liquid such as ethyl alcohol or benzene, as it is obvious that I can use various mixtures of liquids. For example, a mixture of ethyl alcohol and benzene in equal parts may be used, for although this mixture has a very high solvent action on nitrocellulose of about 11.0% nitrogen, the solvent action materially decreases as the nitrogen increases, and on pyro powder there is 85 no solvent action but only slight swelling 90 of the powder grains. Instead of benzene, toluene or xylene or mixtures thereof may be used with the ethyl alcohol or with other alcohols.

The property or properties of the powder 95 which are responsible for the particular viscosity which, in any particular case, the powder imparts to its solutions, may be designated, briefly, the viscosity-characteristic of the powder—the change which the powder undergoes upon heating being accordingly describable as a reduction in its viscosity-characteristic.

My invention may be illustrated by the 100 following example:

A sample of pyro smokeless powder of 3" field gun granulation originally containing 0.45% diphenylamine was heat treated 105

by immersing it in denatured ethyl alcohol containing  $\frac{1}{2}$  gal. benzene to 100 gals. of ethyl alcohol, the denatured alcohol being boiled in a suitable still provided with a 5 condenser for condensing the alcohol and returning same to the still for reuse. The viscosity of the powder was originally 250 seconds in a solvent mixture composed of benzene 50, ethyl alcohol 20, and ethyl acetate 10 30, parts at a temperature of 28° C. by the so-called steel ball method, this time being that required by a  $\frac{1}{2}$ " steel ball to fall through 10" of a solution containing 16 oz. of the powder to 1 gal. of the solvent mixture given above. After heating the powder in boiling ethyl alcohol for about 75 hours, using sufficient alcohol to keep the powder always covered, the viscosity of the powder was reduced to 20 secs. and the content of the diphenylamine, both converted and unconverted, remaining in the powder was less than 0.02%, a practically negligible amount.

During the boiling treatment, the alcohol 25 may be changed several times if extraction of the diphenylamine and its derivatives to a minimum quantity is desired. By unconverted diphenylamine, I mean diphenylamine plus the nitroso-diphenylamine, the latter having been shown by investigators 30 to be almost the equivalent of diphenylamine in its stabilizing action on powder. By converted diphenylamine, I refer to the nitro derivatives of diphenylamine.

35 When the viscosity-characteristic of the pyro powder is originally low, a shorter time of treatment in boiling ethyl alcohol is required in order to reduce the viscosity to a point where the powder is suitable for use 40 in the preparation of pyroxylin solutions. For example, a 30 hour boiling treatment in ethyl alcohol sufficed to reduce the viscosity-characteristic of a sample of pyro powder to such an extent that the viscosity 45 of its solution was reduced from 85 to 20 secs., the content of converted and unconverted diphenylamine remaining in the powder being reduced to less than 0.02%.

I have also discovered that different 50 liquids do not have the same effect in regard to reduction in viscosity, even though they may be used at the same temperature; and that different liquids extract more or less of the diphenylamine and its derivatives. For example, a 30 hr. boiling treatment of the above pyro powder in benzene reduced the viscosity to only 76 secs. while the content of converted and unconverted diphenylamine remaining in the powder 55 was 0.32%. On the other hand, by boiling the same pyro powder in toluene of the commercial grade with a boiling point of approximately 111° C., the viscosity was more rapidly reduced than when boiled in benzene; thus 24 hours of boiling with toluene

sufficed to reduce the viscosity of the particular sample of pyro powder from 85 secs. to 17 secs., the content of converted and unconverted diphenylamine remaining in the powder being 0.41%. After 40 hours 70 boiling with toluene, the diphenylamine content was 0.35% and the viscosity of the solution was 5 seconds.

While it is impossible to remove the last traces of nitro derivatives of diphenylamine, 75 the amount remaining in the powder is so small as to permit the powder to be used in the preparation of pyroxylin solutions where a light color is an important feature. Where the presence of the diphenylamine 80 in the treated powder is not objectionable, I may heat treat the pyro powder in toluene or other liquid or mixtures of liquids which, while effecting only partial extraction of the diphenylamine, will reduce the viscosity of 85 the powder in an economical manner.

In certain cases the reduction of the diphenylamine content is the most important feature of the process, especially 90 where the pyro powder available already possess such a low viscosity characteristic as to require but a slight further reduction. In bringing about this reduction in diphenylamine content, the difference in the effectiveness of an alcohol, such as ethyl alcohol, on the one hand, and of a benzoid hydrocarbon on the other, is remarkable. Treatment of the powder with ethyl alcohol for from 15 to 30 hours serves to remove practically all of the diphenyl- 100 amine, whereas treatment of the powder with benzene or toluene under the same conditions of time and temperature will remove no more than about 25% of the diphenylamine initially present. 105

This greater effectiveness of the alcohol in removing diphenylamine is not due to a greater solvent power possessed by the alcohol for diphenylamine, since the latter is more than twice as soluble in benzene 110 and toluene as it is in ethyl alcohol.

While I prefer, in practicing the process, to maintain the particular liquid employed at or below its boiling point because of the simplicity of apparatus required, it is 115 sometimes expedient to heat the pyro powder in the liquid at temperatures above its normal boiling point, for example between 75 and 135° C., by the use of an autoclave.

In any event, in the heat treatment of the 120 powder, I prefer to use temperatures at which objectionable decomposition of the powder does not take place. If desired, I can heat the powder immersed in the liquid at a temperature of from 55 to 60° C., and depend on a number of days of treatment to reduce the viscosity of the powder to a point where the same is satisfactory for use in the preparation of pyroxylin solutions. I may follow treatment at low temperature with 125 130

treatment at a higher temperature with the same or a different liquid. However, I prefer to use the liquids previously mentioned at or near their boiling points—ethyl alcohol and 5 benzene, for example, at a temperature of approximately 80° C., toluene at a temperature of about 111° C., and xylene at about 135° C. While I prefer not to exceed a temperature of 135° C., in some cases where the 10 powder requires relatively little heat treatment to give it the desired viscosity-characteristic, I may give the powder a very short heat treatment at a temperature above 135° C., but in all events avoiding objectionable 15 decomposition of the powder.

When the powder grains are large in size, for example, more than 1" in length, I prefer to grind or crack the powder to smaller size in suitable grinding apparatus so that 20 smaller sized grains will be available for the heat treating process. This facilitates the extraction of the diphenylamine and its derivatives from the powder, besides facilitating the solution of the powder after the 25 heat treatment is completed. Even when the powder grains are not large, the powder may be first ground to shorten the time required for extraction, but when the original grains are quite small, the decrease in extraction time resulting from preliminarily 30 grinding the powder may be insufficient to justify the added trouble and expense of such grinding. Instead of grinding the powder under water, I preferably grind the 35 powder under ethyl alcohol and either heat the powder in boiling ethyl alcohol, or drain off the alcohol and heat the powder in toluene or in another liquid or mixtures of liquids of the kind above-described.

40 I claim:

1. The process of reducing the viscosity-characteristic of pyro powder containing diphenylamine which comprises heating the powder, immersed in an organic liquid in 45 which the powder is substantially insoluble, at a temperature below 150° C.

2. The process of concurrently reducing the viscosity-characteristic and the diphenylamine content of pyro powder, which comprises heating said powder at a temperature below 150° C. while it is immersed in a liquid which is a solvent for the diphenylamine but a non-solvent for the remainder of the powder. 50

3. The process of reducing the viscosity-characteristic of pyro powder containing diphenylamine which comprises heating the powder at a temperature between about 60 and 135° C. in contact with an organic liquid in which said powder is substantially insoluble, until the desired change in the viscosity-characteristic of the powder has occurred. 55

4. The process of concurrently reducing the viscosity-characteristic and the diphenylamine content of pyro powder, which comprises heating said powder immersed in ethyl alcohol at a temperature between about 75 and 135° C. until the desired change in the viscosity-characteristic of the powder has occurred. 60

5. The process of rendering pyro powder containing diphenylamine suitable for use in light colored coating compositions, which comprises treating said powder with an alcohol until the desired reduction in the diphenylamine content has occurred. 70

6. The process of rendering pyro powder containing diphenylamine suitable for use in light colored coating compositions, which comprises treating said powder with ethyl alcohol until the desired reduction in the diphenylamine content has occurred. 80

7. The process of rendering pyro powder containing diphenylamine suitable for use in light colored coating compositions, which comprises heating said powder with an alcohol at a temperature below 150° C. until the desired reduction in the diphenylamine content has occurred. 85

In testimony whereof I affix my signature. 90

RICHARD G. WOODBRIDGE.